

## UNITED STATES PATENT OFFICE

2,220,059

PROCESS FOR REDUCING CORROSION BY  
AMMONIACAL SOLUTIONS OF INORGANIC  
SALTS AND NEW COMPOSITION OF RE-  
DUCED CORROSIVENESSHerman A. Beekhuis, Jr., Petersburg, Va., and  
Charles K. Lawrence, Baldwinsville, N. Y., as-  
signors to The Solvay Process Company, New  
York, N. Y., a corporation of New YorkNo Drawing. Application June 13, 1938,  
Serial No. 213,452

14 Claims. (Cl. 23—239)

The present invention relates to methods of reducing corrosion of ferrous metals by solutions of inorganic salts in ammoniacal liquors.

In recently developed processes for the ammoniation of superphosphates use is made of solutions containing large percentages of inorganic salts and also free ammonia. Such solutions are in general quite corrosive in their action on ferrous metals. The provision of methods which 0 reduce or prevent the corrosion of apparatus constructed of ferrous metals in which these solutions are handled constitutes a major problem in the commercial use of these solutions, since, when they are shipped in tank cars of the usual 5 construction, rapid corrosion occurs and the tank soon is not usable. Also corrosion occurs in apparatus constructed of ferrous metals in which the solutions are handled.

It is, therefore, an object of the present invention to provide a method for reducing the rate 0 of corrosion of ferrous metals by solutions of inorganic salts in ammoniacal liquors to an extremely low rate.

It is a further object of this invention to provide 5 solutions of inorganic salts in ammoniacal liquors which corrode ferrous metals only extremely slowly.

It is a further object of this invention to provide a method for rendering solutions of inorganic salts, in ammoniacal liquors, which normally corrode ferrous metals rapidly, much less 0 corrosive in their action on said ferrous metals.

In general, ammoniacal solutions of inorganic salts are corrosive with respect to ferrous metals 5 and the process of this invention may be employed to reduce the rate of corrosion of ferrous metals by such solutions. The invention is particularly applicable to ammoniacal solutions of those nitrogenous salts which are employed in the production of fertilizers; for example, solutions of ammonium salts, such as ammonium nitrate and ammonium chloride, or nitrates, such as sodium nitrate and ammonium nitrate; or so- 5 lutions containing ammonium carbonate or carbamate, particularly solutions of urea in ammoniacal liquors which also contain compounds of ammonia and carbon dioxide. Ammoniacal solutions of thiocyanates, such as ammonium thiocyanate, may be treated in accordance with

this invention to reduce the corrosion of ferrous metals contacted therewith.

According to the present invention, the apparatus, which may be a storage tank, tank car, 5 conveying pipe, measuring tank or the like, is constructed of the ferrous metals commonly used for this purpose such as low carbon steels, for example structural steel, cast iron and wrought iron.

In employing this invention a compound of 10 trivalent arsenic is incorporated in a solution of an inorganic salt in an ammoniacal liquor, such as aqua or anhydrous liquid ammonia, particularly an ammoniacal liquor of 5% or greater strength. The trivalent arsenic compound added to the ammoniacal solution (i. e. prior to incorporation in the solution) may be, for example, arsenic trioxide ( $As_2O_3$ ), or a sulfide of trivalent arsenic, for instance,  $As_2S_2$  (realgar) or  $As_2S_3$ , such as precipitated arsenic trisulfide or orpiment, or an arsenite, for instance sodium or ammonium arsenite. In case arsenic trioxide is used, it may be in any of its forms, for instance white arsenic, either crystalline, as octahedral 15 crystals or amorphous, or vitreous arsenic trioxide. The incorporation of a trivalent arsenic compound in a solution of an inorganic salt in an ammoniacal liquor reduces the rate of corrosion of ferrous metals in contact with the solution 20 to an extremely low rate.

Compounds of trivalent arsenic dissolve but slowly when added directly to the ammoniacal salt solutions except at elevated temperatures which, if employed, would necessitate the use of high pressure equipment and the consumption 35 of large quantities of heat. Accordingly, the arsenic compounds are preferably first dissolved in an alkaline solution, such as an aqueous solution of soda ash, caustic soda, ammonia, or the like. Small quantities of the alkaline solution 40 containing arsenic may then be added to the ammoniacal salt solution.

The quantity of arsenic compound added may 45 vary from a very small percentage upward, and may vary with the composition of the salt solution. In general, it is preferred to add the arsenic compound in the amount of about 0.05% or more (calculated as  $As_2O_3$ ). The objects of the invention may be obtained by adding large amounts 50 of the arsenic compounds, although the arsenic

compound in solution will constitute a minor proportion by weight of the total composition and no added advantage is obtained by adding the arsenic compound in excess of the solubility thereof in the particular solution employed. Less than 0.05% may be added, though the protection afforded is not as great as with the preferred amounts.

Our invention has specific application to am-  
10 moniacal solutions of the nitrates, particularly of ammonium nitrate. It appears from our ob-  
servations of the action of numerous salt solu-  
tions on ferrous metal that the chemical reaction  
which causes rapid corrosion of ferrous metals by  
15 ammoniacal ammonium nitrate solutions is pre-  
cious to nitrate solutions and to ferrous metals.  
Further, in the case of the nitrate solutions,  
rapid corrosion of the metal as a result of this  
reaction occurs only with the ammoniacal solu-  
20 tions. Thus, in the case of acid and neutral  
solutions of ammonium nitrate, hydrogen is  
evolved by the corrosion of ferrous metal by the  
solutions. In the case of corrosion by am-  
moniacal ammonium nitrate solutions, instead  
25 of detecting the evolution of hydrogen, we have  
observed that ammonia is formed by reactions  
taking place during corrosion of the metal by the  
solution. Under the conditions encountered in  
the corrosion of ferrous metals by ammoniacal  
30 ammonium nitrate, the presence in the solu-  
tion of even a small amount of a trivalent arsenic  
compound appears to inhibit the particular type  
of corrosion involved.

The preferred ammoniacal solutions of nitrate  
35 to which our invention has specific application  
are aqueous solutions of ammonium nitrate contain-  
ing free ammonia in which the ammonium  
nitrate constitutes about 50% or more of the  
solution (for example, 40% to 80%) and in which  
40 the ammonium nitrate is dissolved in 5% or  
stronger aqua ammonia, particularly in an aqua  
ammonia of about 25% or greater strength due  
to the relatively high rates of corrosion exhibited  
by these solutions.

45 Our invention further has specific application  
to the prevention of corrosion by ammoniacal  
urea-carbonate solutions; that is, ammoniacal  
solutions of mixtures of urea, ammonium car-  
bonate and ammonium carbamate such as may  
50 be produced in conjunction with the synthesis of  
urea. Our preferred urea-carbonate solutions,  
to which the invention relates, may contain be-  
tween about 25% and about 50% urea, between  
about 5% and about 30% of combined ammonia  
55 and carbon dioxide, in the form of ammonium  
carbonate and ammonium carbamate, and the  
remainder an ammoniacal liquor of 5% or greater  
strength. We have found the addition of a  
trivalent arsenic compound, as above indicated,  
60 is very effective in reducing the rate of corro-  
sion of ferrous metals by these solutions.

In order to protect the ferrous metals even  
further, we have found it desirable also to add to  
the solution a compound of the general class of  
65 compounds which contain divalent sulfur linked  
to carbon and preferably linked to an atom of  
carbon with the remaining valences of the car-  
bon atom linking the carbon to nitrogen. As il-  
lustrative of these compounds which further re-  
duce the rate of corrosion, the following are  
70 noted:

- (a) Carbon disulfide ( $S=C=S$ );  
(b) The thio alcohols, such as ethyl mer-  
captan ( $C_2H_5.SH$ ), and benzyl mercaptan  
75 ( $C_6H_5CH_2SH$ );

(c) The thio ethers, such as diethyl sulfide  
[( $C_2H_5$ )<sub>2</sub>S];

(d) The organic thio acids, their salts and es-  
ters, such as:

(1) Thiocyanates ( $X-S-C\equiv N$ ), e. g., ethyl 5  
thiocyanate, alkali metal thiocyanate,  
ammonium thiocyanate, etc.

(2) Derivatives of the thio analogues of  
carbonic acid, such as potassium xan-  
thate 10



(3) Thiocarboxylic acids, such as thioacetic 15  
acid



20

(4) Thiophenols, such as thiophenol  
( $C_6H_5SH$ ), and thio beta naphthol  
( $C_{10}H_7SH$ );

(e) Thioamides such as thiourea [ $(NH_2)_2C=S$ ] 25  
and thioacetamide



30

(f) Heterocyclic compounds containing divalent  
sulfur in the ring such as thiophene



35

and thiadiphenyl amine



40

Compounds containing divalent sulfur linked 45  
to carbon are suitable for use in carrying out  
this invention, but it is preferred to use com-  
pounds in which the remaining valences of the  
carbon atom linked to divalent sulfur are satis-  
fied by one or more atoms of nitrogen such as 50  
the thiocyanates and thiourea.

The quantity of organic sulfur compound 55  
which may be incorporated to reduce the rate of  
corrosion may vary from a very small percentage  
upward. It is preferred, however, that the solu-  
tion contain 0.004% to 0.8% of these materials  
(calculated as sulfur). More than 0.8% (cal-  
culated as sulfur) may be present although the  
presence in the solution of a high proportion of  
the sulfur compounds is not necessary to ac-  
complish the purposes of the invention and the  
amount of the sulfur compound is, in general a  
minor proportion by weight of the amount of the  
total inorganic salt content of the solution. For  
example, any of the materials listed in the pre-  
ceding paragraph may be added, to a solution 65  
containing 60 parts of ammonium nitrate, 20  
parts ammonia, 20 parts water and 0.1% arsenic  
trioxide ( $As_2O_3$ ), in amount corresponding to  
70 0.04% sulfur.

The rate of corrosion of ferrous metals by am-  
moniacal salt solutions varies with the varying  
conditions under which the solutions and metals  
are in contact with each other. The protection  
afforded the metal under some conditions en- 75

countered in commercial shipment and use of the solutions may be materially increased by the addition of the above described sulfur compounds to the solution. Further, the addition of these sulfur compounds serves to protect the arsenic compounds in the solution. Thus, while under most conditions the presence of the arsenic compound alone affords a lasting protection against corrosion, when corrosion does occur a product of the reaction of ferrous metals with ammoniacal solutions of inorganic salts appears to be a ferrous compound which is soluble in the solution but is oxidized by the air to an insoluble ferric compound. This ferric compound is precipitated from the solution and appears to adsorb arsenic compounds. By incorporating in the solution a divalent sulfur compound, removal from the solution of arsenic compound, with a consequent loss in the protective action of the arsenic compound in the solution against corrosion of the metal, may be prevented. Accordingly, the divalent sulfur compounds perform, in conjunction with the arsenic compounds, the double function of protecting the metal against corrosion under varying conditions and of guarding against loss of the protective action of the trivalent arsenic compounds.

*Example 1.*—An alkaline arsenite solution is prepared by dissolving 10 parts octahedral crystalline arsenic trioxide in 90 parts of a 15% aqueous solution of sodium hydroxide at room temperature. One part of the arsenite solution so prepared is added to 100 parts of a solution containing 60% ammonium nitrate, 20% ammonia, and the remainder chiefly water. The solution so produced contains 0.1% arsenite (calculated as  $As_2O_3$ ). The thus treated solution is then contacted with apparatus made of ferrous metal. It has been found that the rates of corrosion of low carbon steel and cast iron contacted with such a solution are extremely low; thus, low carbon steel submerged in the solution was corroded at a rate equivalent to a penetration of only 0.002 inch per year; cast iron at 0.003 inch per year. In a similar solution but containing 0.05%  $As_2O_3$ , low carbon steel is corroded at a rate equivalent to a penetration of 0.003 inch per year.

*Example 2.*—Vitreous arsenic trioxide, commercial white arsenic, orpiment and realgar are individually dissolved in caustic solutions. These solutions are added to ammoniacal solutions of ammonium nitrate as in Example 1. Upon contacting the solutions with low carbon steel apparatus, similar results are obtained as in the above example.

*Example 3.*—To 100 parts of a solution containing 60% ammonium nitrate, 20% ammonia, and 20% water are added 0.1 part ammonium thiocyanate and 0.5 part of an arsenite solution prepared as in Example 1. The solution, which then contains 0.04% ammonium thiocyanate (calculated as sulfur) and 0.05% arsenite (calculated as  $As_2O_3$ ), is then contacted with low carbon steel. Steel contacted with a solution so treated has been found to be corroded at a rate equivalent to an average penetration of less than 0.001 inch per year.

*Example 4.*—50 pounds of commercial white arsenic and 75 pounds soda ash are dissolved in 50 gallons of water at about 95° C. with agitation. The solution so prepared and about 300 pounds of a crude aqueous 33% ammonium thiocyanate solution are added to 45 tons of a solution containing 60% ammonium nitrate, 20%

ammonia, and the remainder chiefly water. The ammoniacal ammonium nitrate solution is then placed in a conventional type tank car for shipment.

*Example 5.*—1 part of an alkaline arsenite solution prepared as in Example 1 is added to 100 parts of a solution containing 33% urea, 17.7% combined carbon dioxide and ammonia, 27.8% free ammonia, and the remainder chiefly water. The solution so prepared contains 0.1% arsenite (calculated as  $As_2O_3$ ). This solution is then contacted with low carbon steel which has been found to be corroded thereby at a rate equivalent to a penetration of less than 0.001 inch per year.

*Example 6.*—1 part of an alkaline arsenite solution, prepared as in Example 1, is added to 100 parts of a solution containing 58% ammonium nitrate, 16% urea, 13% ammonia and the remainder chiefly water. This solution is then contacted with low carbon steel which has been found to be corroded thereby at a rate equivalent to a penetration less than 0.001 inch per year.

We claim:

1. The process of reducing corrosion of a ferrous metal by an ammoniacal solution of an inorganic salt, which comprises incorporating in said solution a trivalent arsenic compound in amount sufficient to decrease the rate of corrosion of a ferrous metal by said solution, and contacting said solution with said ferrous metal.

2. The process of reducing corrosion of a ferrous metal by an ammoniacal solution of an inorganic salt, which comprises incorporating an arsenite in said solution in amount sufficient to decrease the rate of corrosion of a ferrous metal by said solution, and contacting said solution with said ferrous metal.

3. The process of reducing corrosion of a ferrous metal by an ammoniacal solution of an inorganic salt, which comprises incorporating a sulfide of trivalent arsenic in said solution in amount sufficient to decrease the rate of corrosion of a ferrous metal by said solution, and contacting said solution with said ferrous metal.

4. The process of reducing corrosion of a ferrous metal by an ammoniacal solution of an inorganic salt, which comprises incorporating in said solution both a trivalent arsenic compound and a compound containing divalent sulfur linked to carbon in amounts sufficient to decrease the rate of corrosion of a ferrous metal by said solution, and contacting said solution with said ferrous metal.

5. The process of reducing corrosion of a ferrous metal by an ammoniacal solution of an inorganic salt, which comprises incorporating in said solution both a trivalent arsenic compound and an alkali metal thiocyanate in amounts sufficient to decrease the rate of corrosion of a ferrous metal by said solution, and contacting said solution with said ferrous metal.

6. The process of reducing corrosion of a ferrous metal by a solution of ammonium nitrate containing free ammonia, which comprises incorporating in said solution a trivalent arsenic compound in amount sufficient to decrease the rate of corrosion of a ferrous metal by said solution, and contacting said solution with said ferrous metal.

7. The process of reducing corrosion of a ferrous metal by a solution of ammonium nitrate containing free ammonia, which comprises incorporating in said solution both a trivalent arsenic compound and a compound containing divalent sulfur linked to carbon in amounts suffi-

cient to decrease the rate of corrosion of a ferrous metal by said solution, and contacting said solution with said ferrous metal.

8. The process of reducing corrosion of a ferrous metal by a solution of ammonium nitrate containing free ammonia, which comprises incorporating in said solution both a trivalent arsenic compound and an alkali metal thiocyanate in amounts sufficient to decrease the rate of corrosion of a ferrous metal by said solution, and contacting said solution with said ferrous metal.

9. The process of reducing corrosion of a ferrous metal by an ammoniacal solution of urea and a compound of carbon dioxide and ammonia, which comprises incorporating in said solution a trivalent arsenic compound in amount sufficient to decrease the rate of corrosion of a ferrous metal by said solution, and contacting said solution with said ferrous metal.

10. As a new composition of matter of reduced corrosiveness with respect to ferrous metals, an ammoniacal solution of an inorganic salt containing a trivalent arsenic compound in amount sufficient to decrease the rate of corrosion of a ferrous metal by said solution.

11. As a new composition of matter, an ammoniacal solution of an inorganic salt containing a trivalent arsenic compound and a compound containing divalent sulfur linked to carbon in amounts sufficient to decrease the rate of 5 corrosion of a ferrous metal by said solution.

12. As a new composition of matter, an ammoniacal solution of ammonium nitrate containing a trivalent arsenic compound in amount sufficient to decrease the rate of corrosion of a ferrous metal by said solution.

13. As a new composition of matter, an ammoniacal solution of ammonium nitrate containing a trivalent arsenic compound and a compound containing divalent sulfur linked to carbon in 15 amounts sufficient to decrease the rate of corrosion of a ferrous metal by said solution.

14. As a new composition of matter, an ammoniacal solution of urea and a compound of ammonia and carbon dioxide containing a trivalent arsenic compound in amount sufficient to decrease the rate of corrosion of a ferrous metal by said solution.

HERMAN A. BEEKHUIS, JR.  
CHARLES K. LAWRENCE. 25